

Dec. 28, 1954

W. E. KINGSTON ET AL

2,697,869

PROCESS FOR MAKING ALUMINUM COATED MATERIAL

Filed April 23, 1948



FIG. 1



FIG. 2

INVENTORS  
Walter E. Kingston  
Igor N. Zavarine  
Charles E. Bussert  
Brock B. Richardson  
His Attorney

# United States Patent Office

2,697,869

Patented Dec. 28, 1954

1

2,697,869

## PROCESS FOR MAKING ALUMINUM-COATED MATERIAL

Walter E. Kingston, Port Washington, and Igor N. Zavarine, Great Neck, N. Y., and Charles E. Bussert, Middletown, Ohio; said Bussert assignor to Armeo Steel Corporation, a corporation of Ohio, and said Kingston and said Zavarine assignors to Sylvania Electric Products, Inc., New York, N. Y., a corporation of Massachusetts

Application April 23, 1948, Serial No. 22,814

1 Claim. (Cl. 29—189)

The present invention relates to a method of coating metallic stock, and in particular to the production of an adherent iron-aluminum alloy on a ferrous sheet. Advantageously, relatively ductile sheet stock may be produced by the present process, which may be formed and drawn into components for radio tubes.

It is readily possible to coat iron or mild steel sheet or strip stock with aluminum by hot dipping, as by following the methods and using the apparatus of the United States Sendzimir Patent 2,110,893.

Since the processes of this patent include a heat treatment which may be carried on as a softening anneal, the hot coated products, as produced, may be characterized by good formability and good drawability, and the adherence of the aluminum coating is sufficient to permit these operations.

However, for the attainment of certain thin gauges, and for the attainment of certain other gauges with the greatest possible convenience and economy, it is at present found necessary to reduce the thickness of the coated product after it has been coated. Also, as will hereinafter appear, certain final products require a thickness of coating substantially less than the minimum thickness which can at present be applied in hot dipping procedures. In these instances the coated product will be subsequently cold rolled, and it has been found that the coating produced as set forth above readily withstands such cold rolling treatments.

The result of cold rolling will be a work hardening of the iron or steel stock in proportion to the amount of cold work performed on it, and this in turn will ordinary destroy the forming and drawing characteristics of the material. Since practically all products which would be fabricated from such stock would require either drawing or forming, a heat treatment in the nature of a softening anneal is indicated. But a heat treatment at a temperature high enough to produce softening of the iron or steel within a given length of time, will within the same length of time cause the aluminum coating to alloy fully with the metal of the sheet or strip stock.

It has hitherto been suggested that the inclusion of certain elements such as silicon or others in the molten coating metal will, to a degree at least, control the formation of iron-aluminum alloys. Such elements, and others, appear to have a measurable effect in controlling alloying during the formation of a coating by hot dipping, but their effect seems without importance in preventing alloying during a heat treatment practiced upon precoated materials. At least, in our investigations we have not been able, by the addition of any elements to the aluminum in the coating, to produce a substantial softening of a cold rolled iron or steel stock by an annealing treatment at any temperature for a sufficient length of time to produce softening in a commercial fashion without at the same time alloying the aluminum with the iron. The addition of silicon, magnesium, or other substances to the aluminum bath used in coating may be desirable for other reasons, and where herein we refer to aluminum we desire to be understood as including not only the substantially pure metal but also aluminum containing minor amounts of other substances including those mentioned above.

So far as we know, the only successful instances of

5

2

the annealing of iron or steel sheets previously coated with aluminum, carried on in such a way as not to produce alloying, are to be found in the German "Feran" process in which layers of iron and aluminum are joined by rolling together to form a plate which is then reduced to final thin gauge by such an exceedingly great amount of cold work, say a cold reduction of the order of 98 per cent, that recrystallization will occur at an abnormally low temperature. Under these circumstances it has been found possible to produce softening without completely alloying the aluminum with the iron. Such excessive reductions are not economical as they must be carried out on small mills and in small plates, nor do they form part of the processes to which this application relates.

For some uses where a bright surface of aluminum is desired a complete alloying of the aluminum coating with the iron of the base cannot be tolerated. For other uses, the bare fact that an iron or steel product is coated with a coating of aluminum-iron alloy instead of aluminum might not necessarily be disadvantageous. It will be understood that the aluminum-iron alloy so produced is grey or black in color, and for some uses this is desirable. For example, cookie pans and other metal baking trays formed of iron or steel sheet metal having a bright aluminum coating are not satisfactory. By reason of the high heat reflectivity of the coating, insufficient heat is transferred through the pan to the bottom surface of the dough or batter to produce proper cooking on the bottom side within the length of time in which the top surface of the dough is browned by direct radiation from heating elements and from reflection from the pans above. Again, in the formation of anodes for radio tubes a dark surface having a high black body radiation coefficient is required.

It has been generally recognized that the efficiency of certain elements of an electron discharge tube are increased if the surfaces of these elements are blackened so as to increase their heat radiation. It is also generally known that such blackened materials will have a smaller secondary emission as compared to bright materials.

45

It is for these reasons that carbonized nickel, carbonized nickel plated steel and carbonized steel strip material have found general application in the electron discharge tube art particularly for use as an electrode material for those tubes in which a comparatively high heat dissipation is required during operation.

In the case of anodes made from the product of the German "Feran" process it has been the practice to produce by heat treatment an alloying of the aluminum with the iron in the finished, fabricated anodes. Hot dipped aluminum coatings alloyed with the base metal have similarly been found to have excellent black body characteristics which make them suitable for radio tube anodes. It has always been found, however, that when a stock hot-dipped in aluminum has been subsequently cold reduced to a lighter gauge and heat treated sufficiently to soften the base metal and transform the coating completely to iron-aluminum alloy, this alloy is brittle and of poor adherence so that the stock could not be formed or drawn without destroying and flaking away the alloy coating, leaving the base metal unprotected.

While we shall describe our invention in connection with a process involving substantial amounts of cold rolling, it will be understood that in instances where the required thicknesses of the base stock and the required thickness of coating can otherwise be obtained, it may still be desirable to provide a completely alloyed coating prior to forming or drawing, and the invention herein described is not limited to cold rolling except as set forth hereinafter.

The principal objects of our invention lie in the solution of problems briefly discussed above, and other objects, which will be set forth hereinafter or will be apparent to one skilled in the art upon reading the disclosures which follow. The several objects of our invention are attained by that procedure and in that

product of which we shall now describe certain exemplary embodiments.

In the drawings:

Fig. 1 is a photomicroscopic view of an aluminum coated steel strip showing fine surface cracks which do not penetrate to the base metal,

Fig. 2 is a photomicroscopic view of an aluminum coated steel strip showing large surface cracks penetrating to the base metal.

We have discovered that under certain circumstances, hereinafter explained at length, it is readily possible to coat an iron or steel stock with aluminum, then, as may be necessary to obtain the desired thinness of product and coating, cold reduce the coated product, and finally develop desired degrees of drawability or formability therein by a heat treatment which at the same time will produce an alloying of the aluminum with the iron of the base, and that it is also possible to produce thereby a product in which the aluminum alloy layer is so firmly bound to the base that the stock may be subjected to drastic forming operations or to repeated drastic drawing operations without loss or essential disruption of the coating.

The particular requirements which we have discovered must be met in the practice of our process to result in this novel product are:

1. In the final stage of the product, the aluminum-iron alloy coating layer must be very thin—less than certain maximum values.

2. The time and temperature of the heat treatment must be so limited and coordinated that the base metal will be softened and the coating completely alloyed without the formation of non-adherent iron-aluminum alloys.

We shall now take up in detail the requirements for the production of sheet or strip metal of the kind just described.

The base metal sheet or strip stock may be of iron or mild steel, either rimming or killed, as these terms are understood in the art. Other ferrous base metals may be used, however, as this is not a limitation of the invention.

The base metal sheet or strip stock should be coated with a sound and tightly adherent coating of aluminum, which as set forth above may if desired contain minor amounts of other alloying ingredients. The coating is preferably done by the processes and with the use of apparatus set forth in the Sendzimir patents mentioned above, or may be accomplished otherwise.

The aluminum-coated iron or steel strip stock may then be cold rolled to final gauge. In order to meet the maximum coating-thickness requirement, the aluminum-coated product when at final gauge and prior to alloying should bear on any coated face an aluminum coating not greater than substantially between .0003 inch and .0001 inch in thickness, average. The thickness of coating may be determined either by microscopic methods, or by chemical methods in which the average weight of coating per unit area of surface represents a certain thickness.

In the aluminum coated and cold rolled condition a weight of .50 ounce of coating per square foot of sheet is approximately equivalent to a .001" coating thickness on each side of the sheet. Similarly .050 ounce of coating represents .0001 inch thickness. These figures are approximately correct for either pure aluminum or aluminum containing 9 percent silicon. The chemical method of determining the coating thickness by stripping the aluminum coating from the sheet stock before subjecting it to heat treatment at the range at which alloying takes place is a preferred method for determining the thickness of coating.

While somewhat thicker coatings may be employed, the maximum range given is one within and below which a satisfactory adherent and formable or drawable alloy coating can dependably be produced in accordance with our teachings. This is irrespective of the specific final thickness of the base sheet or strip stock, although in certain circumstances the thickness of the coating within the range set forth may advantageously be varied with the thickness of the final gauge of the base stock. By way of example, the thickness of an iron or steel sheet or strip stock intended for use in the fabrication of anodes for radio tubes will be of the order of .005 inch. The thickness of an iron or steel sheet or strip stock intended for fabrication into cookie pans may be of the order of .05 inch. In the case of such thin materials as those

used in radio tubes it has been found that the specific thickness of the ultimate iron-aluminum alloy layer has an appreciable effect on the stiffness of the annealed product. Hence in commercial operations our preference is to manufacture coated sheet or strip stock of the thinner type with aluminum coatings near the lower end of the coating thickness range, while heavier base stocks may be manufactured with aluminum coatings near the higher end of the coating thickness range.

The final annealing or heat treatment which forms the second requirement of our process is very important; but it will be understood by the skilled worker in the art that variations are contemplated depending upon the particular qualities desired in the final material. A cold reduced, coated product will not be very satisfactorily formable or drawable without a softening heat treatment; but formability usually requires a greater degree of softness and a larger grain size than those which produce maximum drawability. The final heat treatment may be in the nature of a box anneal or in the nature of an open or strand anneal, and it may be varied in known ways to obtain the desired characteristics in the base metal, within the limits hereinafter set forth. The softening produced is a function of time and temperature, higher temperatures requiring less time as is well understood. Moreover the rapidity of softening will generally depend upon the percentage of cold reduction practiced on the coated product.

Approximately the lowest feasible temperature for softening the base metal or alloying the coating will be around 1050 degrees F., at which temperature the time required to produce the necessary softness for a forming or drawing stock will be of the order of hours, indicating the practice of a box anneal. As the temperature rises, the time for softening decreases rapidly as does also the time required to cause the aluminum layer to alloy fully with iron from the base. Thus at 1550 degrees F. satisfactory softness and full alloying will occur in a matter of seconds or minutes depending on the thickness of the base metal. For example, we have found that for base metal of .005 inch thickness only 17 seconds are required while for .050 inch thickness approximately 2 minutes are needed. This indicates the feasibility of a strand or open anneal at this and other temperatures down to about 1200 degrees F. below which we have found the required time to be unduly long.

In general excellent results can be attained with the range of coated materials set forth herein by open annealing treatments between substantially 1450° and 1750° F. for times between 7 minutes and 17 seconds.

The qualities of the alloy layer may be impaired by overheating. Thus at temperatures higher than about 1800 degrees F. the alloy coating tends to take on a grayish appearance and to become markedly less adherent.

Microscopic examination leads us to believe that this phenomenon is due to the further diffusion of iron into the alloyed coating with a resultant increase in the thickness of the alloy layer accomplished by a decrease in its adherence. In general, we prefer to confine the annealing temperatures to those not higher than about 1750 degrees F. The qualities of the coating may also be impaired by holding the material for too great lengths of time at lower temperatures. Thus where full alloying occurs in 17 seconds at 1550 degrees F. a strand or open anneal is advisable since a box anneal will unduly prolong the time at which the material is held at high temperature.

Where the time for softening to a desired degree is measured at a particular temperature in hours, we prefer a box anneal; but where a temperature is employed which will produce complete alloying in a time measured in minutes or seconds we prefer an open or strand anneal. The choice of temperatures and times may largely be determined by the desired qualities of the finished product, it being understood that prolonged holding at elevated temperatures promotes grain growth and formability.

By formability as used herein we mean the ability of the sheet or strip stock to take a sharp bend without undue springback, and by drawability we mean the property of the material to become deformed by stretching in suitable drawing dies. While the greatest possible degree for formability, all other conditions being equal, can be attained by prolonged holding at an elevated temperature, satisfactory degrees of formability for most uses can be attained in open or continuous anneals at somewhat higher temperatures.

By an open or continuous anneal is meant a heat treatment in which the material in single thickness sheets or strip form is carried through an elongated furnace.

The atmosphere during the heat treatment is not of controlling importance. Oxidizing atmospheres may be employed especially in continuous or open anneals; but our preference is for an atmosphere of non-oxidizing, inert gas, such as nitrogen, or of any commercially available reducing atmosphere, including hydrogen, dissociated ammonia, the so-called "d-x" gas and many others. It is not necessary in the practice of our process to employ what is commonly known as a bright annealing atmosphere.

Cold rolling of the aluminum-coated iron or steel stock when required may be carried out with any suitable equipment.

In practice with present hot-dipped coatings, cold reduction is required if the aluminum coating is to be made thin enough, and substantial cold rolling is further of advantage in introducing enough strain into the base metal to enable it to be softened at relatively lower temperatures.

In the coating of iron or steel stock with aluminum by hot dipping for our purpose it is highly desirable that the coating be controlled as to uniformity. Moreover, the thicknesses of coatings applied by hot dipping methods are circumscribed and cannot be greatly varied if uniformity is to be achieved. For example, aluminum coatings of controlled uniformity can be applied roughly between .001 and .002 inch in thickness, while wiped coatings, i. e., coatings treated by the wiping means disclosed in U. S. Patent No. 2,398,034 to Oganowski issued April 9, 1946, or by other suitable wiping means, can be made on the order of about .0005 inch in thickness. It will be evident that substantial cold reduction of such a coated product will be required to reduce the thickness of such coatings to the range of substantially .0003 inch to .0001 inch or less set forth above. There is in general a practical upper limit to the thickness of strip stock which may be passed through coating apparatus of the kind referred to above, which lies at around .125 to .150 inch. On the other hand considerations of economy in the use of apparatus and mechanical limitations of the apparatus lie against the coating of exceedingly thin stocks; and in any event it will be found helpful to practice substantial cold work on the coated stocks in order to reduce the thinnest practical coatings to the thickness range required for the production of adherent alloy layers.

It will now be evident that the operator should calculate back from the desired final thickness of base stock and final thickness of aluminum coating to determine a suitable initial thickness of coated stock, initial thickness of coating, and amount of cold reduction required to produce the finished product. However, it is readily possible for final products in which the thickness of the base iron or steel sheet or strip lies roughly between .08 and .005 inch with aluminum layers or coatings lying substantially between .0003 and .0001 inch in thickness to determine the thicknesses of starting sheet or strip suitable for aluminum coating, thicknesses of initial aluminum coatings and degrees of cold reduction to be performed on the coated product which will meet the requirements as set forth herein. By way of example, we now give representative procedures which we may employ in producing satisfactorily softened strip with alloyed coating, where the strips are .005, .05 and .08 inch in thickness.

#### Example 1

Hot roll to .080 inch  
Cold reduce to .040 inch  
Aluminum coat .001 inch each surface  
Cold reduce to .005 inch  
Final aluminum thickness .00013 inch each surface  
Open anneal at 1550 degrees F. for 17 seconds in dissociated  $\text{NH}_3$  atmosphere.

#### Example 2

Hot roll to .180 inch  
Cold reduce to .100 inch  
Aluminum coat and wipe to .0005 inch each surface  
Cold reduce to .05 inch  
Final aluminum thickness .00025 inch each surface  
Open anneal at 1475 degrees F. for 4 minutes in an atmosphere of dissociated  $\text{NH}_3$ .

#### Example 3

Hot roll to .150 inch  
Aluminum coat and wipe to .0005 inch each surface  
Cold reduce to .08 inch  
Final aluminum thickness .00027 inch each surface  
Open anneal at 1475 degrees F. for 7 minutes.

It will be understood that these exemplary procedures are illustrative and not limiting, and that the conditions set forth herein may be attained by substantial departures therefrom. The final heat treatments in the examples above produce the desired adherent coatings and a sufficient softness of the material for forming and drawing purposes as well as the desired adherent blackened coating.

With special reference to electron tube strip it may be said that under present usage, any strip or sheet material prepared for use as electrode material in an electronic tube must be soft enough so that it will not cause excessive wear on the shaping tools; but of far greater importance, it must retain its complex shape (as observed in multitudinous numbers of shapes of anodes) after forming within an extremely close tolerance.

A physical testing machine to describe whether the material meets this specification is the bend tester designated as ASTM-B-155-41T. For the purpose of using our shaping tools, we have found that anode material should have a deflection angle of 35 degrees or less, as measured by this bend tester, and this angle value is specified for material for this use, though some tolerances in this limiting figure, usually up to 40 degrees maximum is allowed for continuous production of material.

The material after cold rolling to the desired size, usually about .005 inch shows a bend test angle considerably greater than 35 degrees regardless of the thickness, percentage of aluminum or percentage of reduction in thickness, and obviously must be softened prior to use. Further, this softening must be consistently duplicable from a production standpoint to allow continuous flow of the material through the anode forming machines.

The following table of bend test values, obtained from a series of .005 inch strip containing varying thicknesses of aluminum alloy, show that it is not possible to bright anneal this strip at or below 1000 degrees F. consistently and reliably to attain the desired bend test.

| Temp., ° F. | .00028" | .00025" | .00033" | .00036" | .0005"  | .0006"  |
|-------------|---------|---------|---------|---------|---------|---------|
|             | Degrees | Degrees | Degrees | Degrees | Degrees | Degrees |
| 50          |         |         |         |         |         |         |
| 900         | 24      | 41      | 43      | 55      | 33      | 43      |
| 950         | 28      | 33      | 32      | 59      | 33      | 47      |
| 1,000       | 28      | 28      | 30      | 39      | 33      | 41      |

The values in inches are for the thickness of the aluminum on strip .005 inch in thickness.

The following table of bend test angles shows that as the aluminum alloy thickness increases, it becomes progressively more difficult to soften the material sufficiently even though the time or temperature be increased.

| Temp., ° F. | Time in Furnace, Minutes | .0005"  | .00033" | .00025" |
|-------------|--------------------------|---------|---------|---------|
|             |                          | Degrees | Degrees | Degrees |
| 65          |                          |         |         |         |
| 1,250       | 4                        | 39      | 32      | 29      |
|             | 2                        | 38      | 32      | 29      |
|             | 1                        | 36      | 33      | 30      |
| 1,350       | 4                        | 41      | 34      | 31      |
|             | 2                        | 38      | 34      | 31      |
|             | 1                        | 38      | 34      | 32      |
| 70          | 4                        | 41      | 35      | 32      |
| 1,450       | 2                        | 39      | 34      | 33      |
|             | 1                        | 39      | 33      | 33      |
| 1,550       | 4                        | 41      | 36      | 31      |
|             | 2                        | 41      | 36      | 32      |
|             | 1                        | 41      | 36      | 30      |
| 75          | 4                        | 39      | 34      | 29      |
| 1,650       | 2                        | 39      | 35      | 29      |
|             | 1                        | 39      | 36      | 28      |

The lower practical thickness of aluminum is determined by the factors of increased gas evolution of the electrode in the electronic tube and by the commercial unfeasibility of cladding steel with very thin layers of aluminum by a hot dip method.

The upper temperature limit for treating the .005 inch strip for use as electrode material is dictated by two

effects. The first of these is as follows: If two pieces of the strip from the same sheet, are simultaneously annealed and blackened, one at 1250 degrees and the other at 1650 degrees, a difference in behaviour with respect to forming properties is noted.

Material transformed (annealed and blackened) at the lower temperature when bent around a sharp radius will show closely spaced, very fine cracks on the surface, none of which penetrate to the base metal. Note Fig. 1 of the drawings which shows a photomicroscopic view of the above-described aluminum clad steel strip. However, the material transformed at 1650 degrees will show widely spaced, wide cracks which penetrate somewhat into the metal. Note Fig. 2 which shows a photomicroscopic view of the aluminum coated strip treated at 1650 degrees F. Material heated to temperatures much above 1650 degrees F. will crack through the strip if exposed to the critical stresses of an electrode forming operation.

The second effect relating to the upper temperature limit is the surface condition of the coating. Deviations from a black body condition cause a decided loss in the radiation characteristics of the electrode, which are of utmost importance to efficient operation of the electronic valve.

We have found the black color of the surface is due to an iron aluminum compound formation coupled with a thin film of black iron oxide, though we do not wish to limit the scope of this invention to the exact nature of the blackened surface. We have found that the blackened surface can be brightened considerably to a light grey by heat treating in a dry hydrogen gas atmosphere (dew-point—minus 30 degrees C.), at 1650 degrees F. or in a less reducing atmosphere at higher temperatures, such as 1700 degrees to 2000 degrees F. Obviously, from an electrode standpoint, this brightening is undesirable. Inasmuch as the heat treating (simultaneous annealing and blackening) is preferably carried out in an easily controllable reducing type atmosphere (as is well known, strongly oxidizing atmospheres tend to form flaky, poorly adherent oxide scales on iron), it may be desirable to restrict the temperature to 1650 degrees F. or below. If the conditions as set forth above are met, a sheet or strip product is produced which is coated with a dark or black layer comprising or consisting principally of an iron-aluminum alloy. It is a discrete layer, very thin, and sharply demarcated from the iron itself. This layer is tough and adherent so that the product may

be formed or drawn repeatedly without flaking of the coating. The iron or steel sheet or strip base stock will have the desired qualities for forming or drawing, and these operations will not affect the integrity of the coating. The product will have the other desirable characteristics set forth hereinabove.

Modifications may be made in our invention without departing from the spirit of it. Having thus described our invention in certain illustrative embodiments, what we claim as new and desire to secure by Letters Patent is:

A process of producing a coated ferrous sheet gauge stock which comprises hot rolling ferrous metal to thicknesses substantially between .180 and .080 inch, cold rolling it to thicknesses substantially between .100 and .040 inch, coating the cold rolled stock with aluminum in thickness substantially between .002 and .0005 inch on any coated surface, cold rolling the stock to thicknesses between substantially .06 and .005 inch whereby to reduce the aluminum coating thereon to between substantially .0003 and .0001 inch on any coated surface and thereafter heat treating the coated stock wherein said heat treatment is an open anneal, the temperatures lying within the range substantially between 1450 and 1750 degrees F. for a time varying directly with thickness of base metal and inversely with temperature between substantially 7 minutes and 17 seconds.

#### References Cited in the file of this patent

#### UNITED STATES PATENTS

| Number    | Name             | Date           |
|-----------|------------------|----------------|
| 1,656,892 | Shover           | Jan. 17, 1928  |
| 1,792,377 | Jordan           | Feb. 10, 1931  |
| 1,877,569 | Falkenthal       | Sept. 13, 1932 |
| 1,982,563 | Wimmer           | Nov. 27, 1934  |
| 2,082,622 | Fink             | June 1, 1937   |
| 2,110,893 | Sendzimir        | Mar. 15, 1938  |
| 2,170,361 | Whitfield        | Aug. 22, 1939  |
| 2,197,622 | Sendzimir        | Apr. 16, 1940  |
| 2,406,245 | Oganowski et al. | Aug. 20, 1946  |
| 2,444,422 | Bradford         | July 6, 1948   |

#### FOREIGN PATENTS

| Number  | Country       | Date           |
|---------|---------------|----------------|
| 210,377 | Switzerland   | Sept. 16, 1940 |
| 526,525 | Great Britain | Sept. 19, 1940 |